

[54] **IRIDIUM-HAFNIUM ALLOY**

1,016,809 1/1966 United Kingdom..... 75/172 R

[75] Inventors: **Henry Inouye; Chain T. Liu**, both of  
Oak Ridge, Tenn.**OTHER PUBLICATIONS**[73] Assignee: **The United States of America as  
represented by the United States  
Energy Research and Development  
Administration**, Washington, D.C.Shunk, "Constitution of Binary Alloys, Second Sup-  
plement," N.Y., McGraw-Hill, 1969, pp. 416-417.[22] Filed: **Apr. 26, 1974***Primary Examiner*—L. Dewayne Rutledge[21] Appl. No.: **464,429***Assistant Examiner*—E. L. Weise  
*Attorney, Agent, or Firm*—Dean E. Carlson; David S.  
Zachry; John B. Hardaway

[52] U.S. Cl..... 75/172 R

[57] **ABSTRACT**[51] Int. Cl.<sup>2</sup>..... C22C 5/04A new iridium alloy comprising up to about 1 weight  
percent hafnium has greatly improved physical and  
mechanical properties as compared to pure iridium.

[58] Field of Search..... 75/172 R, 134 V

[56] **References Cited****3 Claims, 1 Drawing Figure****FOREIGN PATENTS OR APPLICATIONS**

1,051,224 12/1966 United Kingdom..... 75/172 R



## IRIDIUM-HAFNIUM ALLOY

## BACKGROUND OF THE INVENTION

This invention was made in the course of, or under, a contract with the United States Atomic Energy Commission. It relates generally to the metal alloy art and particularly to a new iridium alloy.

As is disclosed in commonly assigned U.S. Pat. No. 3,737,309, isotopic heat sources have found considerable use as both terrestrial and space power sources. The most prominent radioisotope fuels are  $^{238}_{\text{Pu}}$  and  $^{244}_{\text{Cm}}$ . Nuclear emissions from these sources produce heat which is converted into electricity by means of thermoelectric generators or thermionic devices.

Radioisotopic fuels used in space power systems must be encapsulated in a highly reliable material. The encapsulation material must not only be able to contain the fuel for normal operation of several years but also to survive launch abort situations, severe aerodynamic heating on re-entry, high velocity impact, and post impact environment. One alloy developed for such purposes is disclosed in U.S. Pat. No. 3,737,309. While the Pt-Rh-W alloy disclosed therein possesses the requisite mechanical properties for space applications, it tends to react with the fuel at temperatures in excess of 1250°C. Another material considered for use as an encapsulation material is highly purified iridium as is disclosed in U.S. Pat. application Ser. No. 372,886. Purified iridium possesses the necessary high temperature inertness, but it does not have the requisite mechanical properties.

Several prior-art iridium alloys containing W or Nb have been produced. These alloys have been found to confer moderate improvements in the mechanical properties.

## SUMMARY OF THE INVENTION

It is thus an object of this invention to provide a new alloy which is suitable for use as a radioisotope encapsulation material.

It is a further object of this invention to provide an iridium alloy with greatly improved mechanical properties.

These as well as other objects are accomplished by an iridium alloy having 0.3 to 1.0 weight percent hafnium.

## BRIEF DESCRIPTION OF THE DRAWING

The single FIGURE of drawing graphically depicts the toughness of alloys from this invention in comparison with prior-art alloys.

## DETAILED DESCRIPTION

According to this invention it has been found that an alloy of iridium with 0.3 to 1.0 weight percent hafnium has greatly improved mechanical properties as compared to pure iridium while retaining the chemical inertness of pure iridium. Alloys within this range have high toughness, low oxidation rate, high recrystallization temperature, good compatibility with fuels and graphite, and the requisite fabricative properties. The addition of as little as 0.3 weight percent hafnium has been found to be effective to improve the mechanical properties of iridium. The tensile strength, for example, is increased by about 300 percent in alloys containing 0.65 to 0.93 weight percent hafnium. In fact, the mechanical properties tend to improve linearly with in-

creasing amounts of hafnium. However, the fabricative properties are diminished by the hafnium additions, but the alloy remains fabricable up to about 1.0 weight percent. Optimum alloy properties are obtained in alloys containing from about 0.6 to 0.95 weight percent hafnium. The preferred alloy composition contains about 0.65 weight percent hafnium, which is an optimum composition considering mechanical properties and fabricability.

The preferred method of producing the alloy is by electron-beam melting and casting into pancake form or rectangular ingot. The alloy is preferably fabricated by canning the alloy in a molybdenum jacket and hot rolling between 1300° and 1000°C.

While the preferred method of producing the alloy of this invention is to use the highly purified iridium metal produced by the process of copending application Ser. No. 372,886, it is understood that minor amounts of various impurities may also be present. Such impurities may include 20 ppm Al, 10 ppm Cr, 40 ppm Cu, 80 ppm Fe, 10 ppm Ni, 50 ppm Rh, 20 ppm Ta, 30 ppm Th, and 10 ppm oxygen. Intentional addition of up to 1 weight percent zirconium and titanium may also further enhance the mechanical properties of the alloy.

Having generally described the invention, the following specific examples are given as a further illustration thereof, some of which are comparative in nature.

## EXAMPLE I

A 150-gram ingot (1 x 2 x 0.3 in.) of Ir-0.65 wt. % Hf was prepared by electron beam melting and casting. The ingot was clad in molybdenum jackets and hot rolled between 1250° and 1300°C. After a total reduction of 65%, the alloy plate was heat-treated for 1 hour at 1400°C., and then rolled continuously to 0.025-in.-thick sheet at 1100°C. The fabricated sheet had good quality with no indication of surface or end cracks.

## EXAMPLE II

The strength, elongation, and toughness of the Ir-Hf alloys were determined in conventional apparatus at room temperature, 760°C., 1093°C., and 1370°C. The tensile results are shown in Table I and are compared to the values for pure iridium under the same conditions. The strength of the Ir-Hf alloys increases with Hf content and this effect is very prominent at high temperatures. At 1370°C., the alloys containing 0.65 and 0.93 wt. % Hf exhibit tensile strengths ~300% higher than Ir. In fact, these alloys are stronger than all the existing candidate alloys (including refractory alloys) for space isotopic heat sources. The Ir-Hf alloys have excellent ductility at high temperatures as shown in Table I. In FIG. 1, the toughness of Ir-Hf alloys is compared (at 1316°-1370°C.) with Ir, Pt-30 wt. % Rh-8 wt. % W, and refractory alloys. The toughness of Ir-0.65 wt. % Hf is the best and is about 300% higher than unalloyed Ir. Thus, the mechanical properties of Ir alloys containing 0.65 to 0.93% Hf are excellent.

Table I

| Alloy<br>(wt. %) | Mechanical Properties of Ir-Hf Alloy Sheets |            |      |
|------------------|---------------------------------------------|------------|------|
|                  | Strength (in 1000 psi)                      | Elongation |      |
|                  | Yield                                       | Tensile    | (%)  |
| Room Temperature |                                             |            |      |
| Ir               | 8.8                                         | 63.0       | 12.6 |
| Ir-3 Hf          | 21.3                                        | 61.3       | 9.7  |
| Ir-65 Hf         | 30.1                                        | 64.8       | 7.9  |
| Ir-93 Hf         | 43.7                                        | 50.9       | 3.2  |

Table I-continued

| Alloy<br>(wt. %) | Mechanical Properties of Ir-Hf Alloy Sheets |            |      |
|------------------|---------------------------------------------|------------|------|
|                  | Strength (in 1000 psi)                      | Elongation |      |
|                  | Yield                                       | Tensile    | (%)  |
| <u>760°C.</u>    |                                             |            |      |
| Ir               | 12.8                                        | 55.0       | 27.0 |
| Ir-3 Hf          | 14.1                                        | 79.1       | 29.6 |
| Ir-65 Hf         | 21.2                                        | 91.3       | 26.5 |
| Ir-93 Hf         | 30.7                                        | 66.5       | 10.6 |
| <u>1093°C.</u>   |                                             |            |      |
| Ir               | 10.4                                        | 35.1       | 49.4 |
| Ir-3 Hf          | 11.2                                        | 60.9       | 32.5 |
| Ir-65 Hf         | 16.2                                        | 82.1       | 35.7 |
| Ir-93 Hf         | —                                           | —          | —    |
| <u>1370°C.</u>   |                                             |            |      |
| Ir               | 7.5                                         | 22.0       | 41.8 |
| Ir-3 Hf          | 10.3                                        | 44.1       | 43.9 |
| Ir-65 Hf         | 14.7                                        | 61.4       | 50.2 |
| Ir-93 Hf         | 20.0                                        | 65.0       | 40.0 |

## EXAMPLE III

Samples of the Ir-Hf alloy sheets fabricated at 1100°C. were vacuum annealed one hour between 900° and 1600°C. for microstructural examination and to determine the recrystallization temperature. The Ir-0.65 wt. % Hf alloys exhibited no recrystallization at 1150°, 50% recrystallization at 1250°, and complete recrystallization after the 1350°C. treatment. Thus, alloying Ir with 0.65 wt. % Hf increases the recrystallization temperatures by about 400°C. The as-rolled specimens showed fine but elongated grains containing substructure, and the recrystallized ones showed single-phased grained structure. Some indication of a second phase was observed in Ir-0.93 wt. % Hf, but it almost disappeared after an anneal for 1 hour above 1400°C.

## EXAMPLE IV

The oxidation properties of Ir-Hf alloys were investigated by heating specimens, after annealing for 1 hour at 1500°C., in air at a flow rate of 100 liters/hour. The temperatures were 770°C., 870°C., and 1000°C. The results are shown in Table II where they are compared with pure iridium. The oxidation rate of Ir-Hf alloys is lower than that of pure Ir at 770° and 870°, and is comparable at 1000°C.

Table II

| Alloy<br>(wt. %) | Oxidation Rates of Ir and Ir-Hf Alloys<br>in Air Flowing at 100 liters/hr. |                                                          |
|------------------|----------------------------------------------------------------------------|----------------------------------------------------------|
|                  | Oxidation<br>Temperature<br>(°C.)                                          | Oxidation Rate<br>(g cm <sup>-2</sup> hr <sup>-1</sup> ) |
| Ir               | 770                                                                        | $-3.4 \times 10^{-8(a)}$                                 |
| Ir-0.65 Hf       | 770                                                                        | $-2.5 \times 10^{-8(a)}$                                 |
| Ir-0.93 Hf       | 770                                                                        | $+1.0 \times 10^{-8(a)}$                                 |
| Ir               | 870                                                                        | $-1.1 \times 10^{-8(a)}$                                 |
| Ir-0.65 Hf       | 870                                                                        | $-1.0 \times 10^{-8(a)}$                                 |
| Ir-0.93 Hf       | 870                                                                        | $-7.1 \times 10^{-8(a)}$                                 |
| Ir               | 1000                                                                       | $-3.1 \times 10^{-8(a)}$                                 |
| Ir-0.65 Hf       | 1000                                                                       | $-3.3 \times 10^{-8(a)}$                                 |
| Ir-0.93 Hf       | 1000                                                                       | $-3.3 \times 10^{-8(a)}$                                 |

<sup>(a)</sup>Oxidation rate after 1000-hr. exposure.<sup>(b)</sup>Oxidation rate after 330-hr. exposure.

## EXAMPLE V

To characterize the compatibility of Ir-Hf alloys with isotope fueled heat source environments, tensile specimens of Ir-0.93 wt. % Hf were contacted with graphite on one side and exposed to an oxygen pressure of  $1 \times 10^{-5}$  torr at 1300°C. Both sides of the specimens were bright and showed no indication of a reaction after a 1000-hour exposure. The tensile test results are presented in Table III, together with those for unexposed specimens. The exposure to oxygen and graphite did not impair the ductility or the tensile strength of the alloy. Thus, it is concluded that the Ir-Hf alloys are inert to the simulated heat source environment at 1300°C.

15

Table III

| Exposure Time<br>(hrs.) | Tensile Properties of Ir-0.93 wt. % Hf Alloy<br>Exposed to Graphite and Oxygen at 1300°C. |       |                |
|-------------------------|-------------------------------------------------------------------------------------------|-------|----------------|
|                         | Strength (in 1000 psi)                                                                    | Yield | Elongation (%) |
| Room Temperature        |                                                                                           |       |                |
| 0                       | 43.7                                                                                      | 50.9  | 3.2            |
| 1000                    | 41.3                                                                                      | 43.4  | 2.5            |
| <u>760°C.</u>           |                                                                                           |       |                |
| 0                       | 30.7                                                                                      | 66.5  | 10.6           |
| 1000                    | 33.0                                                                                      | 59.4  | 9.4            |
| <u>1370°C.</u>          |                                                                                           |       |                |
| 0                       | 20.0                                                                                      | 65.0  | 40.0           |
| 1000                    | 21.0                                                                                      | 61.3  | 38.0           |

30

## EXAMPLE VI

In order to determine the melting temperature between Ir-Hf alloys and graphite, disk specimens of the Ir-0.93 wt. % Hf alloy were contacted with graphite coupons on both sides and heated rapidly to the desired temperature in a graphite crucible. The results of 10 minutes' heating between 2100° and 2300°C. showed the alloy started to bond with graphite at 2250°C. and to melt incipiently at 2300°C. This demonstrated that the re-entry capability of the Ir-Hf alloys is at least 2250°C.

It is thus seen from the foregoing examples that a new iridium alloy has been developed having greatly improved physical and mechanical properties. While it has been described as an encapsulation for isotopic power sources, many other uses are readily apparent. Such other uses are embodied within the scope of the appended claims.

What is claimed is:

1. An alloy composition comprising 0.3 to 1.0 weight percent hafnium, balance iridium.
2. The alloy of claim 1 consisting essentially of 0.60 to 0.95 weight percent hafnium.
3. The alloy of claim 1 consisting essentially of 0.65 weight percent hafnium, balance iridium.

\* \* \* \* \*

50